

(No Model.)

J. PEDDER.

MANUFACTURE OF PLATES HAVING STRATA OF DIFFERENT METAL.  
No. 350,152. Patented Oct. 5, 1886.



Witnesses.  
C. B. Churchill  
J. Cooke

Inventor.  
John Pedder  
By James D. Ray  
Attorney

# UNITED STATES PATENT OFFICE.

JOHN PEDDER, OF PITTSBURG, PENNSYLVANIA.

## MANUFACTURE OF PLATES HAVING STRATA OF DIFFERENT METAL.

SPECIFICATION forming part of Letters Patent No. 350,152, dated October 5, 1886.

Application filed September 22, 1884. Serial No. 143,636. (No model.)

*To all whom it may concern:*

Be it known that I, JOHN PEDDER, of Pittsburgh, in the county of Allegheny and State of Pennsylvania, have invented a new and useful 5 Improvement in Manufacture of Plates having Different Strata of Metal; and I do hereby declare the following to be a full, clear, and exact description thereof.

My invention relates to the manufacture of 10 plates or bars formed of layers or strata of different metals or metals of different carbons—such as steel plates having centers or backs of iron or soft steel—these plates being largely employed in the manufacture of agricultural 15 implements, where a hard wearing-face is required, and the plate must be tough and strong to resist shocks or blows, or plates having alternating layers of hard and soft metal, these plates being employed in the manufacture of 20 safes, the hard layers to resist boring or cutting tools and the soft layers to resist shocks or blows in breaking into the safe. These plates are formed from ingots or packs, the most approved method of making them from ingots 25 being described in Letters Patent No. 300,730, granted to me June 17, 1884, in which the ingot of combined iron and steel, or of steels of different carbons, is cast in a manner to expose the side edges of the plates inserted in the 30 mold, and the ingot so formed is reduced to plate by flat rolling and edge rolling, and the packs being heated and welded together and subsequently rolled to plate. In casting these ingots in the molds, on account of the warping 35 of the molds and inequalities in the rolled edges of the plates inserted, it is very difficult to prevent the molten steel from running over the side edges of the plates inserted, and in some cases extending entirely across said side 40 edges, and the steel so overlapping the side edges of these plates chills between the plate and the mold, so that in the subsequent rolling of the ingot it does not unite firmly therewith, and, in addition to forming irregular 45 edges, breaks off on slight pressure, leaving depressions in the edges. It is also found that where the plates inserted fit against the side walls of the ingot-mold the molten steel is liable to be chilled by the mold and plate along 50 the edges of the plate, this chill extending into the ingot about one-sixteenth of an inch,

and in some cases, in the subsequent reduction of the ingot to plate, causing an imperfect union along the edges of the several strata of the plate. Where the plates are formed 55 from packs, on account of the difference in ductility of the several plates, it is found almost impossible to weld the packs without causing the overlapping of one layer over another along the side edges of the pack, and in 60 the plate produced by the subsequent rolling the side edges of the several strata are irregular and uneven.

The object of my invention is to overcome 65 these difficulties in the manufacture of these plates.

It consists, essentially, as a step in the art of making these plates, in removing from the ingot or pack the metal overlapping the side edges of the several layers or strata, so as to 70 expose even edges for the subsequent reduction by rolling of the ingot or pack to plate.

It also consists in removing from the ingot the chill formed along the side edges of the strata, so as to expose clean unhardened metal, 75 to unite on the subsequent reduction by rolling of the ingot to plate.

It also consists in certain other improvements, as hereinafter specifically set forth.

To enable others skilled in the art to understand my invention, I will describe the same more fully, referring to the accompanying drawings, in which—

Figures 1 and 2 are views of ingots as cast, and Fig. 3 is a view of a pack as welded, illustrating the manner in which the side edges of the several layers overlap. Fig. 4 is a perspective view of a planer, illustrating the planing of an ingot. Fig. 5 is an end view of a pack, illustrating the planing of the parts 90 overlapping the edges. Fig. 6 illustrates the grinding off of the parts overlapping the edges. Fig. 7 illustrates the cutting or fusing of the parts overlapping the edges. Figs. 8 and 9 illustrate means for cutting or sawing off a 95 portion of the metal cast around the center plate to expose said plate.

Like letters of reference indicate like parts in each.

The ingots shown in Figs. 1 and 2 are formed 100 by inserting into the ingot-mold a plate or plates, *a*, and casting the molten steel *b* around

the plate or plates, the plate shown in Fig. 1 having tapering side edges, as described in application for Letters Patent filed by me February 11, 1884, Serial No. 120,349, and the 5 molds illustrated in said application being preferably employed in casting the ingots.

To secure the plate or plates within the steel and prevent the parting of the ingot when fed to the rolls, the molten steel is cast around the 10 ends of the plate or plates, as shown at *c*, the metal of the outer strata, in thus extending around the ends of the inner stratum or strata, binding the ingot firmly together, while it allows the side edges of all the strata to be exposed to view and substantially even.

On account of the high heat of the molten steel the ingot molds are liable to warp out of shape, and as the plates inserted are rolled to shape and are not absolutely true, there are 15 sometimes small spaces left between the molds and the side edges of the plates, and the molten steel flows into these spaces and is chilled by the mold and plate, the steel thus lapsing over the side edges of the plates inserted, as at *d*. 20 It is also found that the molten steel close to the ingot and the side edges of the plates inserted is sometimes chilled to the depth of about one-sixteenth of an inch along the edges of the plate, and this chilled portion prevents 25 a perfect union of the edges of the rolled plate. The packs formed of layers of metals of different carbons are generally united by heating them and compressing them under a hammer or press, and on account of the difference in 30 ductility of the several plates at a high heat, because of the difference in carbon, the metal of some of the plates passes over the edges of adjoining plates, as shown at *d*, Fig. 3. The overlapping metal and the chill along the edges 35 of the strata may be removed by planing, grinding, cutting, or fusing off by means of a circular saw or any other suitable means. Where the overlapping metal, &c., is planed off, the ingot is placed on the planer *C*, and a portion 40 of the metal along the adjoining edges of the layers or strata is planed off to the depth of about one-fourth inch, thus removing any metal overlapping and also the chilled portion 45 of the edges where the strata meet, thus exposing even side edges of all the strata, so that 50 when the ingot is reduced to plate the edges are distinct and even and a more perfect union formed between the several layers along the edge of the plate. Where the chill and part 55 overlapping are ground off, as in Fig. 6, the ingot or pack is placed on a reciprocating table, *f*, and carried under the revolving emery-wheel *g*, this wheel being supported in a suitable frame, *h*. Where a circular saw is employed, as in Fig. 7, the ingot or pack supported on a reciprocating table is carried in the direction of the line of strata under a rapidly-revolving disk-saw, *k*, and as the saw passes along the line of junction of the strata it cuts

or fuses off any metal overlapping, and at the same time, on account of the high heat generated, fuses the metal and removes the chill of the steel along the line of junction, so that in the subsequent reduction in the rolls the edges are properly united. Any metal extending 70 over the strata may then be knocked off with a hammer. Where the cast steel of the ingot surrounds the side edges of the plate inserted in the mold, as shown at *l*, Figs. 8 and 9, I remove the portions overlapping by a revolving 75 disk-saw or by planing. I prefer to cast these overlapping portions *l* in longitudinal recesses in the mold, so that they extend beyond the body of the ingot, and these overlapping portions *l* can then be sawed off to expose the side 80 edges of the plate inserted, as illustrated in the drawings. I find that by forming a sufficiently thick body of cast steel around the side edges of the plate inserted the chilling along the side edges can be avoided. The ingots or 85 packs, having the metal overlapping the side edges and the chilled portions along said edges removed, as above described, and the side edges of these several strata exposed evenly to view, can then be reheated and rolled to plate or bar by 90 flat and edge or side rolling, and as the edges of the plates in the ingots or packs are even and there is no chilled portion between the edges, the edges of the finished plates will be even, properly united, and free from imperfection.

What I claim as my invention, and desire to secure by Letters Patent, is—

1. As a step in the art of making plates or bars from ingots having strata of different 100 metals, removing from the ingot the metal overlapping the side edges of the several strata to expose even edges for the subsequent reduction of the ingot to plate or bar.

2. As a step in the art of making plates or 105 bars from ingots having strata of different metals, removing from the ingot the chilled portion along the side edges of the several strata to prepare the edges of the strata for proper union on the subsequent reduction of 110 the ingot to plate or bar.

3. As a step in the art of making plates or 115 bars from ingots having strata of different metals, fusing off the chilled portion along the side edges of the ingot to prepare the strata for proper union on the subsequent reduction to plate or bar.

4. An ingot formed of strata of different 120 metals having the side edges of said strata substantially even and the metal of the outer strata extending over the ends of the inner strata, substantially as and for the purposes set forth.

In testimony whereof I, the said JOHN PEDDER, have hereunto set my hand.

JOHN PEDDER.

Witnesses:

JAMES I. KAY,  
J. N. COOKE.